

May 7, 1963

N. M. MATUSEWICZ

3,088,857

TRACER MECHANISM

Filed Nov. 26, 1958



INVENTOR.  
NICHOLAS M. MATUSEWICZ  
BY *R.F. Ross*

ATTORNEYS

1

3,088,857

## TRACER MECHANISM

Nicholas M. Matusewicz, Upland, Calif., assignor to the United States of America as represented by the Secretary of the Navy

Filed Nov. 26, 1958, Ser. No. 776,655

1 Claim. (Cl. 149—38)

(Granted under Title 35, U.S. Code (1952), sec. 266)

The invention described herein may be manufactured and used by or for the Government of the United States of America for governmental purposes without the payment of any royalties thereon or therefor.

This invention relates to a tracer mechanism for use as a target, more particularly, it relates to tracer mechanisms incorporating improved tracer compositions.

The tracer head of this invention is for use as a photoactive source to be attached to rockets and bombs to permit photographing of their trajectories.

A satisfactory tracer head to permit adequate photography for weapon and vehicle evaluation must furnish a trajectory-continuous airborne photoactive source. Additionally, the flare composition used should be one which furnishes maximum continuous luminosity for the weight of the material, as space limitations are obviously critical.

Tracers used in the past have been subject to a number of disadvantages. Previous tracers were of the instantaneous flash type and furnished no time-wise continuity of visibility from point of launch to a desired point of the trajectory of the missile. This is in part due to the fact that previous pyrotechnic formulations used in the tracers contained a fuel-oxidizer system designed to provide oxygen in amounts barely below the point of detonation so that supposedly a composition would be formed providing maximum oxidation without detonation. Theoretical and experimental analysis of these compositions have shown that most of the available oxygen for combustion was not being utilized for this purpose. A further disadvantage of prior art pyrotechnic compositions used in tracers is the fact that they provided low photoactivity to volume ratio due to their chemical composition and the fact that they could not be effectively consolidated. The space in a rocket head which is available for the pyrotechnic composition is quite limited. This accentuates the necessity for a pyrotechnic composition which can be effectively consolidated and which will produce high luminosity for a relatively extended time.

It is therefore an object of this invention to provide a tracer head which furnishes a trajectory-continuous, airborne photoactive source which can be photographed for weapon and vehicle evaluation purposes.

It is another object of this invention to provide a pyrotechnic composition for a tracer head which can be readily consolidated and which provides maximum luminosity over an extended time per weight and volume of the composition.

It is a further object of this invention to provide a pyrotechnic composition for tracer heads in which substantially all of the available oxygen from the oxidizer is utilized for combustion of the fuel present.

It has been found that the above and other objects can be accomplished by the combination of a tracer head of suitable construction; separate ignition means for a pyrotechnic composition; and a pyrotechnic composition comprising an oxidizing agent from the class consisting of nitrates and perchlorates of alkali metals and ammonium, and a fuel comprising a material from the class consisting of magnesium, aluminum, boron and mixtures thereof to which composition has been added a semi-catalytic constituent from the class consisting of man-

2

ganese dioxide, tungstic acid, molybdcic acid, cerium nitrate, thorium nitrate, uranium nitrate, ammonium metavanadate, cerium oxalate, magnesium hydroxide, sodium metaperiodate, magnesium trisilicate, mercuric cyanide, barium peroxide, lithium nitrate, barium nitrate, sodium cobaltinitrite, sodium fluoride, sodium bismuthate, cerrous ammonium nitrate, selenium metal, columbium metal, tantalum metal, and aluminum-calcium alloy.

The invention is best understood by reference to the following description taken in connection with the accompanying drawing which is a horizontal cross-section of the tracer head and firing mechanism for the pyrotechnic composition.

Referring to the drawing, the tracer head is represented generally by the numeral 10 and the consolidated pyrotechnic composition is shown at 11. The tracer head 10 is provided with flame exit ports 12 so arranged and constructed that flames from the burning pyrotechnic will be emitted in a direction perpendicular to the direction of travel of the tracer head. A coating 13 of "first fire" or igniter mixture is painted on the end of the consolidated pyrotechnic composition 11 for ignition of the composition. A spiral 14 of fibrous material impregnated with an ignition mixture containing essentially gunpowder is coated with the "first fire" mixture and sealed to the coating 13. For igniting the "first fire" mixture a conventional type acceleration arming fuze 15 is provided having a spring loaded firing pin which fires a primer which in turn actuates a detonator located in the rotor 18 of the fuze. It will be noted that the forward end of the fuze case is cone-shaped and is so placed with respect to the exit ports 12 as to cause flames to be exited out of the ports. The firing pin, primer and detonator, being conventional, are not shown in detail. The fuze is of the type disclosed in the copending application of Winifred F. Sapp entitled "Rocket Fuze" and filed in the U.S. Patent Office March 12, 1953, under Serial No. 342,039, now U.S. Patent No. 2,948,219. The fuze 15 is mounted in the aft end of the head by means of sleeve 20 and set screw 21. The aft end of the head is provided with threads as shown for attaching the head to a conventional rocket motor used to propel the flare head. The tracer head operates as follows: Upon launch of the rocket or bomb carrying the head, the fuze is armed by acceleration of the missile. Arming of the fuze mechanism releases the firing pin to fire the primer which, in turn, ignites the detonator, the detonator serving as a relay charge to fire the igniter composition and "first fire." The "first fire" upon ignition burns at a temperature sufficiently high to ignite the pyrotechnic composition. The burning of the pyrotechnic mixture creates flames and hot gases which because of their confinement create high pressures. This pressure causes flames to be forced out of the exit ports 12. The pyrotechnic burns for a period of time determined by the amount of pyrotechnic, mesh size of the constituents, consolidation pressures and variations in the formulation. The method and construction for igniting the pyrotechnic composition is not critical but is merely one that has been found to be operative. Other methods may be used. It will be noted that the cone-shaped end of the fuze body 15 provides a baffle adjacent the exit ports 12 for the burning gas and flames from the end-burning pyrotechnic. The cone-shaped end forms a diffuser cone to direct the gases and flames out of the exit ports. The construction and arrangement of the ports and diffuser cone so that the gases and flames are vented at a direction perpendicular to the line of flight and axis of the tracer is an important feature of the invention.

The "first fire" composition used had the following composition:

|                             | Wt. percent |
|-----------------------------|-------------|
| Barium nitrate              | 50          |
| Silicon metal               | 20          |
| Tetranitrocarbazole         | 10          |
| Nitrocellulose or "Laminac" | 5           |
| Zirconium hydride           | 15          |

To this composition sufficient N-butyl acetate was added to make the paste pourable and to permit the first fire to be painted onto the pyrotechnic in a thin layer.

Various pyrotechnic compositions were made up and tested. The basic composition is that of Example I. The additional examples are of compositions made by adding the ingredients shown to Example I. All parts are by weight.

#### EXAMPLE I

The composition consisted of 60 parts of atomized magnesium (-100 to +200 mesh), 40 parts of sodium nitrate (-200 mesh) and 5 parts of "Laminac 4116" added as a binder. This compound gave a candlepower of 400,000.

#### EXAMPLE II

| Additive to Example I                 | Candlepower |
|---------------------------------------|-------------|
| 2½ parts MnO <sub>2</sub> (-200 mesh) | 430,000     |

#### EXAMPLE III

|                                        |         |
|----------------------------------------|---------|
| 2½ parts of Cerium Oxalate (-100 mesh) | 435,000 |
|----------------------------------------|---------|

#### EXAMPLE IV

|                                                     |         |
|-----------------------------------------------------|---------|
| 2½ parts of Antimony Potassium Tartrate (-100 mesh) | 340,000 |
|-----------------------------------------------------|---------|

#### EXAMPLE V

|                                       |         |
|---------------------------------------|---------|
| 2½ parts of lead peroxide (-100 mesh) | 360,000 |
|---------------------------------------|---------|

#### EXAMPLE VI

|                                      |         |
|--------------------------------------|---------|
| 2½ parts of ferric oxide (-200 mesh) | 440,000 |
|--------------------------------------|---------|

#### EXAMPLE VII

|                                 |         |
|---------------------------------|---------|
| 2½ parts potassium permanganate | 390,000 |
|---------------------------------|---------|

#### EXAMPLE VIII

|                                                                                   |         |
|-----------------------------------------------------------------------------------|---------|
| 2½ parts of a mixture of 90 parts of thorium dioxide and 10 parts of cerium oxide | 350,000 |
|-----------------------------------------------------------------------------------|---------|

#### EXAMPLE IX

|                                                               |         |
|---------------------------------------------------------------|---------|
| 2½ parts of thorium dioxide and 2½ parts of manganese dioxide | 400,000 |
|---------------------------------------------------------------|---------|

#### EXAMPLE X

|                               |         |
|-------------------------------|---------|
| 2½ parts of tungsten trioxide | 425,000 |
|-------------------------------|---------|

#### EXAMPLE XI

|                                                                 |         |
|-----------------------------------------------------------------|---------|
| 2½ parts of tungsten trioxide and 2½ parts of manganese dioxide | 415,000 |
|-----------------------------------------------------------------|---------|

#### EXAMPLE XII

|                                 |         |
|---------------------------------|---------|
| 2½ parts of molybdenum trioxide | 450,000 |
|---------------------------------|---------|

#### EXAMPLE XIII

|                                                                |         |
|----------------------------------------------------------------|---------|
| 2½ parts of molybdenum trioxide and 2½ parts manganese dioxide | 450,000 |
|----------------------------------------------------------------|---------|

#### EXAMPLE XIV

|                                                 |         |
|-------------------------------------------------|---------|
| 2½ parts cerium oxide                           | 455,000 |
| EXAMPLE XV                                      |         |
| 2½ parts of cerium oxide and 2½ parts manganese | 455,000 |

The composition range of Example I is as follows:

|                | Wt. percent |
|----------------|-------------|
| Sodium nitrate | 35-45       |
| Magnesium      | 54-64       |
| "Laminac 4116" | 1-2         |

15 Compositions were made and tested in which sodium nitrate of the above composition was replaced by each of the following oxidizing agents: potassium nitrate, ammonium nitrate, ammonium perchlorate and potassium perchlorate. Compositions were made and tested in which the magnesium in the above compositions was replaced by the following:

|                    | Parts by Weight | Wt. percent | Mesh   |
|--------------------|-----------------|-------------|--------|
| Magnesium-aluminum | (60-40)         | 35-45       | 40-600 |
| Magnesium-boron    | (75-25)         | 25          | 40-200 |
| Aluminum-boron     | (80-20)         | 35-25       | 40-400 |
| Boron              | 35-25           | 200         |        |
| Aluminum           | 35-25           | 200-600     |        |

30 To all of the above compositions the following semi-catalytic modifying agents were added within the range of 1 to 10 percent by weight and tested; the additives were added to obtain controlled effects in the catalytic action on burning of the tracer compositions: manganese dioxide, tungstic acid, molybdc acid, cerium nitrate, thorium nitrate, uranium nitrate, ammonium nitrate, ammonium metavanadate, cerium oxalate, magnesium hydroxide, sodium metaperiodate, magnesium trisilicate, mercuric cyanide, barium peroxide, lithium nitrate, barium nitrate, sodium cobaltinitrite, sodium fluoride, sodium bismuthate, cerous ammonium nitrate, selenium metal, columbium metal, tantalum metal, aluminum-calcium alloy. All of the compositions produced a continuous burning flare with good luminosity. The incorporation of the semi-catalytic constituent in the pyrotechnic increases the amount of oxygen liberated during burning, thereby permitting more complete combustion of metal fuels and thus producing a higher luminosity per unit volume. The "Laminac 4116" in the above compositions may be replaced by a nitrocellulose binder with equally good results. Other binders which may be used in equal amounts are fluorocarbon waxes, such as, Kel-F waxes. The amount of binder used is somewhat critical as too much produces too much carbon which takes a prohibitive amount of oxygen from the oxidizer thus resulting in the production of smoke only.

55 "Laminac 4116" is an unsaturated polyester dissolved in a reactive monomer. The monomer is styrene. The polyester is of relatively low molecular weight and is manufactured from one of the group of unsaturated dibasic acids, such as maleic and pumaric acid, and from one of the group of saturated dibasic acids, such as phthalic, isophthalic, and adipic acid; and from one or more from a group of polyols, such as ethylene glycol, propylene glycol, and dipropylene glycol. The polyester solution is a liquid with a specific gravity of 1.10, a viscosity of 4 poises and an acid number of from 10 to 30.

60 The pyrotechnic mixture is prepared as follows: the dry ingredients are blended for thirty minutes in a Lancaster counter-current rapid batch mixer. The binder is then added and blending is continued for one hour. The blended mixture is then screened through a 20 mesh screen, placed in shallow trays and oven cured at 90° F. for 72 hours. The cured mixture is rescreened through

a 20 mesh screen and is then ready to be loaded into the pyrotechnic case 10. The pyrotechnic composition is loaded as follows: with the pyrotechnic case 10 placed in a fixture to prevent permanent deformation of the case under consolidation loads, the pyrotechnic formulation is pressed into the case in two increments of approximately 150 grams each, using 100,000 p.s.i. on each increment.

An ignition mixture, not shown, may be coated on the end of the consolidated pyrotechnic and the "first fire" mixture 13 applied to it. The composition of the ignition mixture may be as follows: 50 percent by weight of a mixture consisting of 90 percent by weight of barium chromate (-325 mesh) and 10 percent by weight of boron (-325 mesh), and 50 percent by weight of a mixture of 50 parts by weight of the pyrotechnic mixture and 5 parts by weight of "Laminac 4116."

Obviously many modifications and variations of the present invention are possible in the light of the above teachings. It is therefore to be understood that within the scope of the appended claims the invention may be practiced otherwise than as specifically described.

What is claimed is:

A pyrotechnic composition screened through a 20 mesh screen consisting essentially of 35 to 45 percent sodium nitrate; from 54 to 64 percent magnesium; and from 1 to 2 percent nitrocellulose binder.

References Cited in the file of this patent

UNITED STATES PATENTS

|           |                      |               |
|-----------|----------------------|---------------|
| 594,594   | Bostwick -----       | Nov. 30, 1897 |
| 613,021   | Schwartz -----       | Oct. 25, 1898 |
| 1,025,500 | Wieser et al. -----  | May 7, 1912   |
| 2,035,509 | Schladt -----        | Mar. 31, 1936 |
| 2,149,314 | Schladt -----        | Mar. 7, 1939  |
| 2,410,801 | Audrieth -----       | Nov. 12, 1946 |
| 2,700,603 | Hart et al. -----    | Jan. 25, 1955 |
| 2,829,596 | Loedding -----       | Apr. 8, 1958  |
| 2,868,129 | Johnson et al. ----- | Jan. 13, 1959 |
| 2,968,542 | Brock -----          | Jan. 17, 1961 |

OTHER REFERENCES

Military Explosives, TM9-1910 TO11A-1-34, April 1955, pp. 276, 287, and 294.